

## UNITED STATES PATENT OFFICE

1,924,168

## ALLOY OF ALUMINUM AND BERYLLIUM

Joseph Kent Smith, Detroit, Mich., assignor to  
Beryllium Development Corporation, New York,  
N. Y., a Corporation of Delaware

No Drawing. Application December 22, 1931  
Serial No. 582,656

2 Claims. (CL 75—1)

This invention relates to alloys in which aluminum predominates, and to which alloys of other metals, beryllium particularly, are added not only to better strength and other mechanical characteristics, but also to at once lower the specific gravity of the alloy and to effect greater resistance to atmospheric corrosion and similar influences.

It has long been known that the addition of beryllium to aluminum results in an alloy which is considerably lighter than is pure aluminum itself, the lessening of weight varying linearly with the beryllium content. At the same time, the resistance to corrosion is considerably improved as beryllium content increases.

Because of the relatively high cost of beryllium, it is frequently desirable to keep the proportion of this element as low as possible, yet not sacrifice its valuable strengthening effects. For this reason, I have sought for metals which would intensify the effects of beryllium when alloyed with a preponderating amount of aluminum, and this invention relates only to those alloys in which the quantity of aluminum exceeds that of beryllium.

I have found that, by the addition of relatively small quantities of molybdenum and/or manganese, in quantities themselves insufficient to increase the specific gravity of the alloy significantly, the effect of beryllium is magnified, and the resulting alloy has materially greater strength, workability, castability, bendability, as well as resistance to corrosion, than the simple binary alloy possesses. In general, I prefer compositions in which the content of aluminum and beryllium is at least ninety-eight percent, with the aluminum running from about 55% to about 70%, the beryllium from about 25% to about

40%, with the remainder manganese and/or molybdenum from a substantial fraction to about 1% each.

The manganese and/or molybdenum, as well as the beryllium for alloys low in beryllium, may be added as a master alloy, alloyed with any convenient percentage of aluminum. The manganese and/or molybdenum may also be added directly to an aluminum-beryllium alloy previously made in any of the standard manners, or the final alloy can be formed by reduction of convenient manganese and/or molybdenum compounds directly by the previously-formed binary aluminum-beryllium alloy.

The ternary or quaternary alloys made in accordance with this invention are particularly well suited for castings requiring strength beyond that of ordinary aluminum, or even of its stronger alloys, like duralumin. They are also well adapted for use in sheet form, as in the case of airplane wings or fuselage parts, or wherever else the combination of ultra-lightness, strength and bendability without breaking is essential.

The percentages are by weight.

I claim:—

1. A beryllium aluminum alloy containing aluminum from about 55% to about 70%, beryllium from about 25% to about 40%, and the balance, not in excess of approximately 2%, molybdenum to harden the aluminum eutectic.

2. A beryllium aluminum alloy containing aluminum from about 55% to about 70%, beryllium from about 25% to about 40%, the two together constituting about 98% of the total, and the balance, not in excess of 2%, being molybdenum to harden the aluminum eutectic.

JOSEPH KENT SMITH.

10

95

5

100

0

105

5

110